

## UNITED STATES PATENT OFFICE

GEORGE A. RICHTER, MILTON O. SCHUR, AND ROYAL H. RASCH, OF BERLIN, NEW HAMPSHIRE, ASSIGNORS TO BROWN COMPANY, OF BERLIN, NEW HAMPSHIRE, A CORPORATION OF MAINE

## PAPER TOWEL AND PROCESS OF PRODUCING THE SAME

No Drawing.

Application filed April 28, 1926. Serial No. 105,330.

This invention has relation to absorptive paper products, and is more specifically concerned with the manufacture of paper towels.

Among the prime qualities desirable in a paper towel are high absorptive capacity and high wet strength. It is further desirable that treatment to increase the wet strength of the towel should not lower its absorptive capacity. Inasmuch as the wet strength of a towel can be increased only at the sacrifice of its absorptive capacity by the use of such sizing material as aluminum resinate, paraffin, oil, rubber, or the like, it usually contains little, if any, sizing material. Consequently, when wetted with water, it immediately undergoes a material loss in strength. Even a relatively strong towel made from kraft or sulphate pulp, upon vigorous wiping with wet hands tends to undergo tearing or disintegration, because of its low wet strength.

The object of the present invention is to produce a towel having a wet strength materially higher than the strength of the usual non-sized towel, without, however, appreciably affecting its water absorptive capacity. We have found that this object may be attained if the fibers are uniformly treated with material from which cellulose may be regenerated, and the cellulose then regenerated on the fibers. The cellulose may be regenerated in situ on the fibers by precipitation from a solution of a suitable cellulose derivative, e. g., viscose, so that the fibers of the towel are bonded together and encased therein. The ability of regenerated cellulose to increase the wet strength of the towel, but without substantially affecting its absorptive capacity, may best be explained by the fact that a cellophane sheet made from viscose absorbs water when submerged therein, but does not disintegrate, and loses approximately only 30% of its initial strength upon saturation.

The towel of the present invention may be produced by various methods of procedure. Thus, a waterleaf paper or web, after it has been formed and dried on the paper machine, in one case is passed through a solution of viscose. Preferably, a dilute solution is employed, so that it may readily pass into the

pores and interstices of the web. The web may be completely dried or else partially dried by evaporating excess water contained therein, and then passed through a suitable setting bath, e. g., a solution of sodium bisulphite and sulphuric acid, thereby effecting a precipitation of regenerated cellulose on all the fibers of the web. The web may then be washed substantially free of acid, steeped, if desired, in a sulphide-removing bath (e. g., sulphurous acid), again washed, dried, and cut up into towels. A towel thus made and containing regenerated cellulose, which encases or covers the fibers and bonds them intimately together, has a materially increased wet strength. The method may be controlled so that about 2% regenerated cellulose is present in the finished towel, which is rendered tough and very strong without material effect upon its water absorptivity, as the incorporation of 2% regenerated cellulose does not fill the pores and interstices of the web to a material extent. Of course, the percentage of regenerated cellulose present in the finished towel is subject to variation. In any event, however, the method is carried out so that individual fibers are encased in and bonded together. The method, however, is subject to some variation. Thus, the step of evaporating moisture from the web after its immersion in a viscose solution may be omitted, as the web may be passed into a setting or precipitating bath immediately after such immersion.

Another method of producing cellulose in a towel web may be carried out like the usual beater-sizing process. For instance, viscose is added to the towel-making stock in the beater engine, preferably after it has been beaten and is then uniformly disseminated throughout the stock by the beater engine. Regenerated cellulose may then be precipitated on the stock by the addition of a suitable precipitating agent, e. g., an acid, acid mixture, or acid salt, whereupon the stock may be washed, if desired, prior to formation into a web. The stock is then run over a papermaking machine, formed into towel material, finished, and cut into towels.

If desired, the viscose may be produced in

55

60

65

70

75

80

85

90

95

100

the web from the web itself, and then precipitated in the web in the form of regenerated cellulose. Thus, the web from the paper machine is passed through a bath of caustic soda of mercerizing strength, similar to that ordinarily used in viscose preparation. The web is then passed through squeeze rolls to remove therefrom any excess caustic soda solution and to produce therein the concentration of caustic soda and cellulose (soda cellulose) desired for conversion into viscose. The fibers of the web may thus acquire only a coating or surfacing of soda cellulose, so that upon passage of the web through a bath of carbon bisulphide or through an atmosphere thereof, viscose is formed on the exterior of the fibers. This procedure also does not materially affect the absorptivity of the web, as the pores and interstices therein are preserved in a substantially unobstructed condition, substantially only the surface of the fibers being affected. The web is then passed through a setting or precipitating bath to effect the precipitation of regenerated cellulose from the viscose, whereupon it is washed free of acid content and finally dried.

Cellulose may also be regenerated in the towel web from other cellulose derivatives. For instance, the web may be passed through a solution of cellulose nitrate in a suitable nitrocellulose solvent, e. g., an ether-alcohol mixture. The solvent may then be evaporated from the web, thus leaving a film of cellulose nitrate on the web and on the individual fibers thereof. The cellulose may then be regenerated from the nitrocellulose in situ on the fibers, by passing the web through an aqueous denitrating solution of sodium sulphide, ammonium sulphide, or other suitable denitrating compound. The denitrated web may then be washed and dried. This procedure, however, is less desirable, inasmuch as it calls for the use of organic solvents.

The cellulose may further be regenerated from a cuprammonium cellulose solution, rather than from viscose. Generally, however, the process may be carried out more expeditiously and more economically by regeneration from viscose.

The presence of regenerated cellulose in a towel web, while advantageous when mechanical pulp, sulphite pulp, or a mixture thereof is used as a raw material, is particularly advantageous when sulphate or kraft pulp is employed as the raw material. A kraft or sulphate towel having regenerated cellulose present therein possesses characteristics departing materially from a like untreated towel which undergoes a marked loss in strength when wetted. A kraft towel containing regenerated cellulose, for instance, does not undergo disintegration and is torn with relative difficulty, even if it is vigorously wiped or rubbed with wet hands and is very tough, strong, and highly absorbent. Prefer-

ably, the towel is crinkled or otherwise roughened at a suitable point in its manufacture, to improve its "wiping" quality.

We are aware of the fact that viscose has been proposed for use as a size for paper, but it should be noted that the present invention involves the presence of regenerated cellulose in a paper towel without any sizing or loading materials, that is, a waterleaf paper towel, so as to increase its wet strength while maintaining a high absorptive capacity. We do not, therefore, claim broadly a paper having regenerated cellulose incorporated therein.

We do not herein claim the subject matter of our application Serial No. 140,676, filed October 9, 1926, which is directed to the conditioning of cellulose fiber, and more especially of a high alpha cellulose wood fiber, for conversion into cellulose derivatives, especially the nitrates, and which involves incorporating a cellulose derivative into such fiber before effecting the conversion of such fiber into cellulose derivatives.

What we claim is:

1. A non-waterproofed paper towel, containing about 2% regenerated cellulose encasing and bonding together the fibers thereof.

2. As an article of manufacture, a highly absorptive crinkled paper towel composed of kraft fiber containing regenerated cellulose imparting sufficient wet strength to the towel so that it will not disintegrate when wiping wet hands.

3. A process of making paper towels having improved wet strength and wiping characteristics, which comprises treating an unsized sheet of kraft paper with a material from which cellulose may be regenerated while maintaining substantially its original absorptivity, regenerating the cellulose in the sheet, and crinkling the sheet.

In testimony whereof we have affixed our signatures.

GEORGE A. RICHTER.  
MILTON O. SCHUR.  
ROYAL H. RASCH.

110

105

115

120

125

130